

## UNITED STATES PATENT OFFICE

1,932,639

## MAGNET CORE

Philip Norton Roseby, Liverpool, England, assignor to Automatic Electric Company Limited, Liverpool, England

No Drawing. Application July 27, 1932, Serial No. 625,208, and in Great Britain July 30, 1931.

7 Claims. (Cl. 175—21)

The present invention relates to the construction of magnet cores and is particularly concerned with the manufacture of cores of the type made from powdered material by the application of high pressure which find considerable application in loading coils as applied to a telephone transmission line. The object of the invention is to produce an improved core of this type by the use of a special alloy and also by 10 the use of an insulating film with more satisfactory properties than those employed hitherto.

According to one feature of the invention, the magnetic particles from which the core is pressed consist of an alloy of iron, nickel and cobalt, for instance in the proportions of 60% iron, 20% nickel and 20% cobalt, or 60% iron, 25% nickel and 15% cobalt.

According to another feature of the invention the insulating film which is necessary to separate the particles from one another consists wholly or mainly of a metallic fluoride which has the valuable property that its insulating qualities are not impaired by the heat treatment which with the alloy considered is desirable after pressing and also that it is able to withstand satisfactorily the high pressures employed in forming the coil.

In order that the invention may be better understood a description will be given of a preferred method of carrying it into effect which is generally similar to that described in my patent specification No. 1,850,181 in connection with a nickel-iron alloy. According to this process, an alloy of iron, nickel and cobalt in the proportions of 60%, 20% and 20% or 60%, 25% and 15% is drawn out into wire of a diameter of the order of 4 mils, and this is then chopped into small lengths, for instance  $\frac{1}{2}$ ". The chopped wire is heated to a temperature of approximately 900° C., and is then cooled in air moderately quickly, for instance by distributing it on a copper plate. The wire particles are then placed in a rotating metal drum with sufficient hydrofluoric or hydrofluosilicic acid solution to wet the particles. Heat is applied and the temperature is gradually raised to approximately 300° C. whereupon the chemical reaction which takes place is substantially complete and the particles are then coated with a film consisting wholly or mainly of metallic fluoride. The particles are now mixed with a suitable quantity of a binder, for instance powdered magnesia, are subjected to a magnetic alignment process for instance as described in my application Serial No. 498,694 filed 28th November 1930, and are pressed in a ring mould. After the pressing operation the cores are heated to a temperature of 450—500° C. which operation serves to increase considerably the permeability of the cores and to reduce 60 the hysteresis loss.

It may be mentioned that the percentages given above for the composition of the alloy are only approximate and also that in some circumstances it may be desirable to add a small percentage of an element such as silicon, tantalum or chromium in order to increase the specific resistance. 65

What I claim as new and desire to secure by Letters Patent is:

1. A magnet core for loading coils or the like 70 in which the finely divided magnetic particles from which the core is pressed are separated from one another by a coating of metallic fluorides.

2. A process for making magnet cores for loading coils or the like in which finely divided particles of an alloy of iron, nickel and cobalt are treated with hydrofluosilicic acid and subsequently subjected to high pressure. 75

3. A process for making magnet cores for loading coils or the like in which finely drawn wire of an alloy comprising approximately 60% iron, 20% nickel and 20% cobalt is chopped into small lengths and treated with hydrofluosilicic acid 80 and subsequently subjected to high pressure. 85

4. A process for making magnet cores for loading coils in which finely drawn wire of an alloy comprising approximately 60% iron, 20% nickel and 20% cobalt is chopped into small lengths, heated to approximately 900° C. and 90 after cooling treated with hydrofluoric acid with gradually increasing temperature up to approximately 300° C. after which the particles are mixed with a binder such as powdered magnesia subjected to a magnetic aligning process pressed 95 to cause them to agglomerate and subsequently heated to a temperature of approximately 500° C. to improve the magnetic properties of the resulting core.

5. A process for making magnet cores for loading coils or the like in which finely divided particles of an alloy of iron, nickel and cobalt are treated with hydrofluoric acid and subsequently subjected to high pressure. 100

6. A process for making magnet cores for loading coils or the like in which finely drawn wire of an alloy comprising approximately 60% iron, 20% nickel, and 20% cobalt is chopped into small lengths and treated with hydrofluoric acid and subsequently treated to high pressure. 105

7. A process for making magnet cores for loading coils or the like in which finely drawn wire of an alloy comprising approximately 60% iron, 20% nickel, and 20% cobalt, to which is added a small proportion of an element to increase the 115 specific resistance, is chopped into small lengths, treated with hydrofluoric acid and subsequently subjected to high pressure.

PHILIP NORTON ROSEBY. 12